

## UNITED STATES PATENT OFFICE

1,984,841

AGENT FOR POLISHING, SHARPENING, AND  
GRINDING ARTICLES OF GREAT HARD-  
NESS

Reinhold Reichmann, Berlin, Germany, assignor  
to Siemens & Halske, Aktiengesellschaft, Sie-  
mensstadt, near Berlin, Germany, a corpora-  
tion of Germany

No Drawing. Application May 25, 1933, Serial  
No. 672,808. In Germany May 30, 1932

4 Claims. (Cl. 51—279)

My invention relates to an agent for polishing, sharpening and grinding articles of great hardness, particularly hard alloys.

Silicon carbide belongs to the class of the 5 hardest grinding materials extensively in use. It is employed, particularly in grinding the so-called hard alloys and metallic carbides which are known in the market under various names. The 10 good grinding effect as a result of the great hardness of the silicon carbide is, however, impaired due to the fact that the crystals are united by means of an argillaceous binding agent, the strength of which is very slight as compared to the strength of the crystals. The crystals are 15 easily pulled apart when machining very hard materials, and the structure is subjected to deterioration, thus causing not only a considerable wear of the grindstones but also reducing the grinding efficiency to a minimum.

20 The object of my present invention is, therefore, to employ as polishing and grinding agent for articles of great hardness the purest possible beryllium oxide sintered at a temperature above 1700° C.

25 Beryllium oxide has hitherto been employed chiefly in the manufacture of refractory crucibles. However, its adaptability as polishing and grinding agent for articles of great hardness has not been recognized heretofore. The use of beryllium 30 oxide in the form of solid bodies such as grindstones and the like is of particular advantage. In this case the particles of the beryllium oxide may be united by a material which is also sintered at a high temperature, such as aluminium 35 oxide. However, a still more compact structure is attained if only the pure particles of beryllium oxide are shaped, for instance with the aid of

a moldable slip or by pressing and if the resulting bodies are sintered at a temperature above 1700° C., for instance, between 1900° C. and 2000° C. If the sintering process is continued for a sufficiently long time at a high temperature 5 the body is considerably solidified by the coalescence of the crystals.

The bodies obtained in the above described manner may not only be utilized for grinding hard metallic alloys and similar materials but 10 they also lend themselves to the grinding and polishing of articles consisting of sintered metallic oxides, for instance, highly sintered aluminium oxide, which owing to its great hardness, 15 could hardly be machined in the past. The agent, 15 however, may also be utilized in a pulverized form.

I claim:

1. An agent for polishing, sharpening and grinding articles of great hardness, particularly hard alloys, a material consisting chiefly of the 20 purest possible beryllium oxide sintered at a temperature above 1700° C.
2. As an article of manufacture, a molded abrasive body of predetermined shape consisting of purest possible beryllium oxide sintered at a 25 temperature above 1700° C.
3. The process of forming an abrasive body of the class described, which consists in taking finely divided pure beryllium oxide, forming therefrom a moldable slip, shaping said body from 30 said slip, and sintering said body at a temperature between 1900° C. and 2000° C.
4. An abrasive material consisting principally of sintered beryllium oxide of a high degree of 35 purity.

REINHOLD REICHMANN.